

## UNITED STATES PATENT OFFICE

2,512,891

## SPINNING ARTIFICIAL MATERIALS

James Wotherspoon Fisher, Edward William Wheatley, and Harold Bates, Spordon, near Derby, England, assignors to Celanese Corporation of America, a corporation of Delaware

No Drawing. Application April 1, 1949, Serial No. 85,047. In Great Britain May 5, 1948

4 Claims. (Cl. 18—54)

1

This invention relates to improvements in spinning artificial materials, and is a continuation in part of our U. S. application S. No. 784,306, filed November 5, 1947.

U. S. application S. No. 784,306 describes the modification of poly-1,2,4-triazoles by reacting them with an aldehyde. This treatment has the effect of insolubilising the polymers and/or rendering them infusible. It is stated that the treatment is preferably applied to the polymers after they have been shaped to the desired form, for example formed into fibres, filaments, bristles and films.

We have now found that such treatments with aldehydes may be applied during the actual formation of the filaments, fibres, bristles or the like by a wet spinning process, and furthermore that the presence during the spinning operation of the aldehyde very much facilitates the actual spinning process.

Formaldehyde is the preferred aldehyde as it reacts fairly readily in the cold and still more readily when heat is applied. This is of importance as the actual time of contact of the filaments or other materials with the precipitating bath is relatively short. Thus, for example, using formaldehyde we have obtained good filaments by spinning a 33% solution in acetic acid of a polyaminotriazole obtained according to U. S. application S. No. 609,031 filed August 4, 1945, by heat treatment of sebacic dihydrazide in presence of hydrazine, the polymer having an intrinsic viscosity of about 0.6, into a coagulating bath consisting of an aqueous solution of caustic soda containing formaldehyde. The rate of spinning should be correlated with the rate of reaction of the formaldehyde. Thus if both the spinning dope and the coagulating bath are at room temperature, low spinning speeds should be used in order to give the formaldehyde time to react in the coagulating bath, so that the filaments on emerging from the bath have sufficient strength. However, by heating either the spinning dope or the coagulating bath or both, higher spinning speeds may be achieved. We have successfully used coagulating baths consisting of a solution of 4% caustic soda and 4% formaldehyde in water at room temperature, and also coagulating baths containing 1% of caustic soda and 0.2—0.5% formaldehyde at raised temperatures, for example temperatures of 40—80° C., either of the dope alone or of both dope and coagulating bath.

The filaments, after formation in the above manner, may be drawn out (the process usually

known as cold drawing). Preferably this drawing operation is carried out while heating the filaments, for example by contact with a hot plate. The filaments should not, of course, be heated to a temperature near the melting point of the polymer.

The following examples illustrate the invention:

*Example 1*

A spinning bath 9 feet in length, 9 inches wide and 6 inches deep was charged to a depth of 4½ inches with a coagulating bath consisting of 4% caustic soda and 4% formaldehyde in water. A spinning jet unit consisting of stainless steel was mounted so as to extrude into the bath and was charged with a solution of a polyaminotriazole obtained according to Example II of British Specification No. 612,609 in 99% aqueous acetic acid, the concentration being 33% by weight. Using a single hole spinning jet of 0.2 mm. and extruding under a nitrogen pressure of 300 lbs. per square inch, a continuous monofil was spun at the rate of 2 metres per minute, the monofil being collected on a hanking machine. The yarn so produced had elastic-like properties and was of low lustre.

*Example 2*

Example 1 was repeated using a multi-hole jet with 0.1 mm. holes. The yarn was similar in appearance and nature to the monofil obtained according to Example 1.

*Example 3*

Example 2 was repeated using a coagulating bath consisting of 2% caustic soda and 2% formaldehyde dissolved in water. After spinning, the yarn was drawn out to about 200% of its initial length while passing over a hot plate. The resulting yarn had a tenacity at break of 1.25—1.3 grams per denier and an extension of 80%.

*Example 4*

Example 2 was repeated using a coagulating bath containing 1% of caustic soda and 0.25% of formaldehyde in water. Again the yarn produced was very easily cold drawn and showed a tenacity at break of 1.8 grams per denier and 170% extension.

*Example 5*

Example 4 was repeated but in this case the spinning solution was raised to 80° C. by passing steam through a jacket surrounding the spinning unit. The coagulating bath was maintained at

25° C. The extrusion rate of the yarn was 6 metres per minute. The resulting yarn showed a higher lustre than that produced in the preceding examples.

*Example 6*

A 30% solution of the same polymer was made up in 99% acetic acid and spun into a bath of 1% caustic soda and 0.25% formaldehyde in water, using a multi-hole jet the holes of which were 0.1 mm. in diameter. In this case the spinning solution and the bath were both maintained at 45-50° C. and the spinning speed was 30 metres per minute. The resulting filaments had a soft texture and a higher lustre than those of the preceding example.

Having described our invention, what we desire to secure by Letters Patent is:

1. Process for the production of artificial filaments, bristles and films, which comprises spinning a solution of a linear polymer containing in its structural unit the 4-amino-1,2,4-triazole ring in acetic acid into an aqueous coagulating bath containing caustic soda and formaldehyde.

2. Process for the production of filaments, bristles, films and the like, which comprises spinning a solution of a linear polymer containing in its structural unit the 4-amino-1,2,4-triazole ring in acetic acid into an aqueous bath containing caustic soda and formaldehyde each in a concentration up to 4%.

3. Process for the production of filaments, which comprises spinning a solution of a linear polymer containing in its structural unit the 4-amino-1,2,4-triazole ring in acetic acid into an aqueous bath containing caustic soda and formaldehyde each in a concentration up to 2%.
4. Process for the production of filaments, which comprises spinning a solution of a linear polymer containing in its structural unit the 4-amino-1,2,4-triazole ring in acetic acid into an aqueous bath containing caustic soda in a concentration of about 1% and formaldehyde in a concentration of 0.2-0.5%, the spinning solution and the coagulating bath being at a temperature of 40-80° C.

JAMES WOTHERSPOON FISHER.  
EDWARD WILLIAM WHEATLEY.  
HAROLD BATES.

20

REFERENCES CITED

The following references are of record in the file of this patent:

UNITED STATES PATENTS

25 Number Name Date  
2,384,369 D'Alelio Sept. 4, 1945

FOREIGN PATENTS

30 Number Country Date  
2,36,297 Germany July 1, 1911